# EUROPEAN PATENT SPECIFICATION

(11) **EP 0 161 245 B1**
(45) Date of publication and mention of the grant of the patent: **25.07.1990**
(21) Application number: 83903870.0
(22) Date of filing: 07.11.1983
(51) Int. Cl.: G01S 7/38, G21K 1/10, G21F 1/10, H01Q 17/00

(54) **LOW DENSITY, ELECTROMAGNETIC RADIATION ABSORPTION COMPOSITION**
ABSORPTIONSZUSAMMENSETZUNGEN NIEDRIGER DICHTE FÜR ELEKTROMAGNETISCHE STRAHLUNG
COMPOSITION A ABSORPTION DE RAYONNEMENTS ELECTROMAGNETIQUES A FAIBLE DENSITE

(43) Date of publication of application: 21.11.1985
(73) Proprietor: THE DOW CHEMICAL COMPANY, Midland Michigan 48640-1967 (US)
(72) Inventor: SOLC, Jitka, Midland, MI 48640 (US); HARRIS, Robert, Francis, Midland, MI 48640 (US)
(74) Representative: Hann, Michael, Dr.
(86) International application number: US8301747
(87) International publication number: WO8502265

(56) References cited:
- EP-A- 0 043 040
- US-A- 2 544 391
- US-A- 2 610 250
- US-A- 3 843 593
- US-A- 3 981 844
- US-A- 4 024 318
- US-A- 4 116 906
- N, Chemical Engineering, "Characteristics of Fine Particles" Issued 11 June 1962. See page 207

## Description

This invention relates to a composition for suppressing electromagnetic radiation and, particularly, for reducing the reflection of microwave energy.

The use of materials for absorbing electromagnetic radiation is wide spread in the coating of (1) military devices which are required to avoid or minimize detection by radar, (2) appliances that employ microwave radiation, and (3) reflectors of ships, airplanes, building and bridges to reduce reflection that often causes navigational errors.

Many materials including natural ones and synthetic ones are known for their ability to suppress electromagnetic radiation in the microwave frequency range. This ability to suppress electromagnetic radiation enables the absorbing material to dissipate electromagnetic energy within the material, thereby reducing the reflection of microwaves.

Of the various absorbing materials, the artificial dielectrics are the most commonly employed. Artificial dielectrics are generally formed by dispersing a magnetic powder or other natural absorber in a dielectric material, such as plastics including thermoplastics and thermosets, ceramics, waxes and the like. The artificial dielectrics which have been formed by loading the aforementioned dielectric binders with magnetic metals, semi-conductors, ferromagnetic oxides or ferrites have very desirable magnetic and dielectric properties.

The use of solid ferrites, i.e., ferromagnetic ferrites formed of ferric oxide and other bivalent metal oxides, as sheet materials for reflecting surfaces and objects to suppress or substantially reduce the reflection of electromagnetic energy offers many advantages.

It has been found that mixed ferrites often provide good absorptive materials over a wide range of microwave frequencies. In addition, ferrites in the form of solid coatings display the higher permeabilities which are required for broad band operation. Such solid ferrite coatings are capable of higher permeabilities than those exhibited by the ferrite powders since the amgnetic properties of ferrite decline appreciably by grinding it into powder form. Thus, it is found that ferrites that are both non-conductive and ferromagnetic provide within a single composition the potentially optimum dielectric and magnetic properties.

From US-A-4,024,318 a filled plastic composition is known which is suitable for use as a radar shield. The composite comprises a first layer of a thermosetting polymer filled with particles of aluminum, iridium, tin, lead, bismuth or elements from Group IIB to Group VIIB of the Table of Elements and a second layer of polymer filled with oxides of these metals. The metal concentration is from 40-93% by weight and the metal oxide concentration is from 40-90 weight percent. The particle size of the filler is from 0.1 to 30 pm. It is also possible to mix the metal and the metal oxide in the same polymer prior curing. The polymer is nonpolar in character.

Unfortunately, it is found that, in the conventional absoptive coatings that contain ferrites, substantial quantities of the heavy ferrites is required in order to achieve the desired absorptive capability. The resulting dense coatings of such conventional absorbers are generally undesirable because they are heavy and difficult to fabricate.

In view of the aforementioned deficiencies of the prior art materials for absorbicg electromagnetic radiation, it is highly desirable to provide a light-weight absorptive material that can be readily fabricated into any shape or applied as a coating to any of a variety of substrates which coatings contain relatively low concentrations of the heavy magnetic particles needed for absorption.

An electromagnetic absorption composition having a density less than 6 g/cm³ comprising a dielectric matrix having dispersed therein magnetic additives characterized in that the magnetic additives comprise
(1) colloidal-size polymer encapsulated particles of superparamagnetic material as an absorber for electromagnetic radiation and
(2) the magnetic particles having a diameter of greater than 1 µm as an attenuator for electromagnetic radiation.

The present invention is such a low density ELM absorption composition which exhibits high efficiency in the absorption of electromagnetic radiation, particularly at microwave frequencies. Such composition (hereinafter called ELM compositions) comprises (1) a dielectric material (hereinafter called dielectric matrix) having dispersed therein (2) a colloidal-size particulate of a material capable of absorbing electromagnetic radiation (hereinafter called ELM absorber) and (3) a particulate of a metal-containing material capable of providing increased attenuation of electromagnetic radiation (hereinafter called ELM attenuator). The concentration of ELM absorber in the ELM composition is advantageously sufficient to provide a magnetic loss tangent greater than 0.05 at a frequency of 2 Gigahertz (GHz) and a composition thickness of 2 centimeters (cm). The concentration of ELM attenuator is sufficient to provide the ELM composition with an attenuation of greater than 0.5 decibels per centimeter (dB/cm) under the aforementioned conditions. For the purposes of this invention, a low density ELM composition has a density less than 6 grams per cubic centimeter (g/cm³). Surprisingly, the low density ELM composition of the present invention exhibits dissipative properties higher than would be expected at the concentrations of ELM absorber being employed.

The composition according to this invention can be used as base for a stable fluid dispersion of the aforementioned ELM attenuator and colloidal-sized particles of the dielectric matrix containing colloidal or sub-colloidal particles of the ELM absorber. Surprisignly, such a dispersion can be applied as a coating and dried to form a continuous film wherein the particles of the ELM absorber are maintained in an essentially discrete spaced apart relationship by the dielectric matrix. Preferably, particles of the ELM attenuator are also substantially maintained in an essentially discrete spaced apart relation by the dielectric matrix.

The ELM composition of this invention is particularly effective as an electromagnetic radiation absorber in such applications as paints and coatings to be used for reflection reduction for metal structures such as towers, bridges, ships, etc.; microwave camouflage and radar camouflage; coatings for appliances wherein microwave radiation absorption is desired, such as in microwave ovens and microwave browning devices: applications related to the transport of solar energy from space satellites; and the like. This ELM composition is also well suited for molding shaped articles and for fabrication into foams and fibers.

### Detailed description of illustrative embodiments

The low density ELM composition of the present invention has a density, an attenuation and a magnetic loss tangent as defined hereinbefore. Preferred compositions have (1) densities in the range from 1.2 to 5, most preferably from 1.5 to 3, g/cm³; (2) magnetic loss tangent greater than 0.1, most preferably greater than 0.2 under the conditions specified hereinbefore; and (3) attenuation greater than 1 dB/cm, most preferably greater than 2 dB/cm.

The ELM compositions comprises three essential components: (1) a dielectric solid matrix acting as the continuous phase for the composition, (2) a particulate ELM absorber that is maintained in an essentially discrete, spaced apart relationship by the matrix and (3) a particulate ELM attenuator. In preferred ELM compositions, the ELM attenuator is also essentially totally dispersed in the dielectric matrix.

The dielectric matrix is suitably any normally solid material capable of serving as an insulating matrix (binder) for the ELM absorber. Preferably, it has an electrical resistivity greater than 106 ohms per centimeter (ohms/cm), more preferably greater than 10" ohms/cm, most preferably from 10¹⁵ to 10²⁰ ohms/cm. Examples of such suitable dielectrics include glass, ceramics, waxes, plastics, including thermoplastics and thermosets, rubber polymers and the like, with the synthetic plastics being preferred. Of the synthetic plastics, preferred are polymers that are water-insoluble and are prepared from hydrophobic monomers that are essentially water-immiscible, i.e., the monomer forms a separate phase when 5 grams of the monomer is mixed with 100 grams of water. Such water immiscible monomers will polymerize under emulsion polymerization conditions to form a water-insoluble polymer which will exist in the form of a stable aqueous colloidal dispersion, usually with the aid of suitable surface active. agents.

The ELM absorber is a material (1) which absorbs electromagnetic radiation having frequencies in the range from 0.3 to 20 GHz and (2) which is in .the form of a colloidal or sub-colloidal size particulate. Preferred ELM absorbers can be further characterized as paramagnetic or superparamagnetic due to their small size. Examples of such materials are compounds of magnetic metals such as ferromagnetic oxides of ferrities, e.g., Fe₃0₄, as well as ferromagnetic ferrites formed of ferric oxide and various bivalent metal oxides such as metal oxides of nickel, zinc and manganese; magnetic metals such as iron, cobalt and nickel and their alloys; and other known ELM absorbing materials such as carbon black, graphite and the like. The ELM absorber generally contains particles having a maximum dimension less than about 1 pm, preferably in the range from about 0.01 to 0.7 pm. Of these materials, the magnetic metallic compounds are preferred, with Fe₃0₄ being most preferred.

The ELM attenuator is preferably a ferromagnetic material which is capable of providing microwave attenuation as described hereinbefore. The ELM attenuator is in the form of particles having a dimension greater than 1 pm, preferably in the range from 1.5 to 100 pm, most preferably from 2 to 75 um. Examples of such attenuating materials are iron, cobalt, nickel, and other ferromagnetic metals as well as alloys of such metals. Of these materials, metallic iron is preferred, with carbonyl iron being most preferred. It is understood, however, that in addition to carbonyl iron, metallic iron made by other procedures such as electrolytic iron, reduced iron and atomized iron are preferred.

In the preparation of the low density, ELM absorbing compositions of this invention, it is advantageous to disperse the ELM absorber into the dielectric matrix such that dielectric matrix forms a continuous phase that maintains the particles of ELM absorber in an essentially discrete, spaced apart relationship. Any of a variety of conventional blending procedures for incorporating a colloidal or sub-colloidal particulate into dielectric binders are suitably employed for this purpose. Preferably, however, the dielectric matrix having the ELM absorber dispersed therein (hereinafter called dielectric/absorber), is prepared by initially forming an aqueous dispersion of the ELM absorber by contacting colloidal or sub-colloidal particles of said absorber with an aqueous solution of a water-soluble surfactant or emulsifier, thereby forming the dispersion which contains from 5 to 70 weight percent of the absorber particles. Examples of preferred aqueous dispersions of ELM absorbers are the so-called ferrofluids such as disclosed in the US-A-3,981,844, preferably those having an average particle diameter in the range from 0.05 to 0.1 micrometer. Preferably, such fluids are aqueous dispersions of the magnetic metals which are stabilized by the presence of surfactants, emulsifiers and/or chemical dispersants as described hereinafter.

Typically, suitable surface active agents, dispersants or emulsifiers include salts of fatty acids such as potassium oleate, metal alkyl sulfates such as sodium lauryl sulfate, salts of alkyl aryl sulfonic acids such as sodium dodecylbenzene sulfonate, polysoaps such as sodium polyacrylate and alkali metal salts of methyl methacrylate/2-sulfoethyl methacrylate copolymers and other sulfoalkyl acrylate copolymers, and other anionic surfactants such as the dihexyl ester of sodium sulfosuccinic acid; nonionic surfactants such as the nonionic condensates of ethylene oxide with propylene oxide, ethylene glycol and/or propylene glycol; and cationic surfactants such as alkylamine-guanidine polyoxyethanols, as well as a wide variety of micelle generating substances described by D. C. Blackley in Emulsion Polymerization, Wiley and Sons, Chapter 7 (1975) and other surfactants listed in McCutcheon's Detergents and Emulsifiers, 1980 Annual North American Edition, McCutcheon, Inc., Morristown, N. J. Also included among the suitable surfactants are the surface active polymers (often called polysoaps), e.g., those described in US-A-3,965,032. Of the suitable surfactants, the anionic varities such as the potassium salts of functionalized oligomers, e.g. Polywet varieties sold by Uniroyal Chemical, are preferred. Such surface active agents or emulsifiers are employed in amounts sufficient to provide a stable dispersion of the ELM absorber in water. Preferably, such surface active agents are employed in concentrations in the range from 0.2 to 10, most preferably from 1 to 6, weight percent based on the aqueous phase. Particularly desirable processes for forming such aqueous colloidal dispersions of the ELM absorber are described in US-A-(s), 3,826,667; 3,981,844; 3,843,540 and Industrial Engineering Production and Research Development, Vol. 19, 147-151 (1980).

The aqueous dispersion of the ELM absorber is then combined with the water-immiscible monomer as described herein to form the desired emulsion by normal mixing procedures, for example, by passing both the dispersion and monomer through a high shear mixing device such as a Waring blender, homogenizer or ultrasonic mixer. Alternatively and preferably, the monomer is added continuously to the aqueous dispersion of the ELM absorber during the polymerization. Advantageously, the monomer is in the form of an aqueous emulsion of the monomer which emulsion is maintained by a water-soluble monomer and/or a water-soluble emulsifier such as described hereinbefore. As another alternative, the aqueous emulsion of the ELM absorber and water-immiscible monomer can be prepared by adding colloidal or sub-colloidal particles of the ELM absorber to an existing aqueous emulsion of monomer. In such instances, it is often desirable to add additional emulsifer or surfactant to the emulsion prior to or simultaneous with the addition of the particles of the ELM absorber. In the emulsion of the ELM absorber and water-immiscible monomer in water, the aqueous phase is present in a proportion sufficient to be the continuous phase of the emulsion. The ELM absorber is present in proportions sufficient to provide the dielectric/absorber particulate with the desired dissipative properties. The water-immiscible monomer is present in proportion sufficient to enclose or encapsulate the ELM absorber when polymerized. The emulsifier and/or surface active agent is present to provide an aqueous colloidal emulsion which is sufficiently stable to be subjected to emulsion polymerization conditions. Preferably, the emulsion contains from 0.1 to 25 weight percent of ELM absorber, from 1 to 30 weight percent of monomer and a remaining amount of the aqueous phase including emulsifier (surfactant), catalyst and the like.

Examples of suitable water-immiscible monomers that can be employed to prepare the aforementioned dielectric/absorber include monovinylidene aromatic monomers such as styrene, vinyl tolune, t-butyl styrene, chlorostyrene, vinyllbenzyl chloride and vinyl pyridine; alkyl esters of σ,8-ethylenically unsaturated acids such as ethyl acrylate, methyl methacrylate, butyl acrylate and 2-ethylhexyl acrylate; unsaturated esters of saturated carboxylic acids such as vinyl acetate, unsaturated halides such as vinyl chloride and vinylidene chloride; unsaturated nitriles such as acrylonitrile; dienes such as butadiene and isoprene; and the like. Of these monomers, the monovinylidene aromatics such as styrene and the alkyl acrylates such as butyl acrylate are preferred.

In addition to the aforementioned water-immiscible monomer, relatively minor portions, e.g., less than 10, preferably less than 5, weight percent based on total monomer component, of a water-soluble monomer such as an ethylenically unsaturated carboxylic acid or its salt such as acrylic acid or sodium acrylate; methacrylic acid, itaconic acid and maleic acid; an ethylenically unsaturated carboxamide such as acrylamide; vinyl pyrrolidone; hydroxyalkl acrylates and methacrylates such as hyroxyethyl acrylate, hydroxypropyl acrylate and hydroxyethyl methacrylate; aminoalkyl esters of unsaturated acids such as 2. aminoethyl methacrylate; epoxy functional monomers such as glycidyl methacrylate; sulfoalkyl esters of unsaturated acids such as 2-sulfoethyl methacrylate; ethylenically unsaturated quaternary ammonium compounds such as vinylbenzyl trimethyl ammonium chloride may be employed. It is critical in the practice of this preferred embodiment,that such water-soluble monomers not be employed in amounts sufficient to render the resulting polymer soluble in water. Particularly effective monomer recipes for the pracice of this invention are those containing from 20 to 90 weight percent of styrene, from 10 to 80 weight percent of alkyl acrylate such as butyl acrylate and from 0.01 to 2 weight percent of the unsaturated carboxylic acids such as acrylic acid, with said weight percentages being based on the weight of total monomers.

The emulsion polymerization conditions employed in the practice of this preferred embodiment of the invention are generally those of conventional free-radical type polymerizations carried out in the presence of a radical initiator such as a peroxygen compound, an azo catalyst, ultraviolet light and the like. Preferably, such polymerization is carried out in the presence of a water-soluble peroxygen compound at temperatures in the range from 50° to 90°C. The emulsion is generally agitated during the polymerization period in order to maintain adequate feed transfer. The concentration of catalyst is normally in the range from 0.005 to 8, preferably from 0.01 to 5, weight percent based on total monomer. Examples of suitable catalysts include inorganic persulfate compounds such as sodium persulfate, potassium persulfate, ammonium persulfate; peroxides such as hydrogen peroxide, t-butyl hydroperoxide, dibenzol peroxide and dilauroyl peroxide; azo catalysts such as azobisisobutyronitrile, and other common free-radial generating compounds. Also suitable are various forms of free-radical generating radiation means such as ultraviolet radiation, electron beam radiation and gamma radiation. Alternatively, a redox catalyst composition can be employed wherein the polymerization temperature ranges from 25° to 80°C. Exemplary redox catalyst compositions include a peroxygen compound as described hereinbefore, preferably potassium persulfate or t-butyl hydroperoxide and a reducing component such as sodium metabisulfite and sodium formaldehyde hydrosulfite. It is also suitable to employ various chain transfer agents such as mercaptans, e.g., dodecyl mercaptan; dialkyl xanthogen disulfides; dialyl disulfides and others listed in Blackley, supra, Chapter 8 in concentrations as described therein.

Following emulsion polymerization, the resulting aqueous dispersion of the particles of dielectric/ELM absorber can be withdrawn from the polymerization vessel nd (1) the dispersion is employed as is or (2) the unreacted monomer and other volatiles are removed to form a concentrated dispersion and then used as a paint base for the ELM composition or (3) the dielectric/ELM absorber particulate can be separated from the aqueous continuous phase of the dispersion by conventional means such as spray drying or drying under vacuum. If dried, the dielectric/ELM absorber particulate preferably contains from 10 to 80, most preferably from 15 to 70, weight percent of the ELM absorber and from 90 to 20, most preferably from 85 to 30, weight percent of dielectric matrix polymer.

In this preferred embodiment, the dielectric/ELM absorber in the form of an aqueous dispersion or a dry colloidal-size particulate is then combined with the ELM attenuator to provide the desired low density, ELM absorbing composition. Preferably, the ELM attenuator (particulate) is dispersed as an aqueous dispersion of the dielectric/ELM absorber, thereby forming a coating composition which can be applied to any substrate as desired and dried to a continuous coating capable of absorbing ELM radiation. Alternatively, the ELM attenuator may be encapsulated in a suitably dielectric material as defined hereinbefore prior to combination with the dielectric/ELM absorber. In this alternative embodiment, the ELM attenuator and dielectric/ELM absorber may be in the form of aqueous dispersions and/or in the form of dry powders when combined.

In dry form, the resulting low density, ELM compositions can be fabricated into an article of desired shape by conventional fabrication techniques such as injection or compression molding, extrusion and the like. Alternatively, the ELM composition in the form of a dry powder is dispersed in a nonaqueous liquid and employed as desired, e.g., as a paint base for other coating formulations.

Preferred low density, ELM absorbing compositions that employ colloidal-size Fe₃0₄ as the ELM absorber and carbonyl iron as the ELM attenuator have an ELM absorber:ELM attenuator weight ratio from 90: 10 to 40:60, most preferably from 80:20 to 55:45. in the preferred ELM compositions, the weight ratio of the sum of ELM absorber and ELM attenuator to the dielectric matrix is from 85:15 to 10:90, most preferably from 70:30 to 55:45. In addition to the foregoing critical components, these compositions optionally contain other ingredients such as stabilizers, pigments, fillers, blowing agents, corrosion inhibitors and other additives commonly employed in ELM absorbing compositions.

The following examples are given to illustrate the invention. Unless otherwise indicated, all parts and percentages are by weight.

### Example 1

### A. Preparation of aqueous dispersion of Fe₃0₄ (ELM absorber)

An aqueous dispersion of magnetic iron oxide (Fe₃0₄) (ELM absorber) is prepared by mixing aqueous solutions of ferric and ferrous salts in amounts to maintain the Fe⁺³/Fe⁺² molar ratio at -2:1. Magnetic iron oxide is then precipitated at 0°-10°C by rapid addition of 1N NH₄0H and vigorous agitation until a pH of 9-10 is reached. Immediately thereafter, the dispersant is introduced with agitation to the aqueous medium containing the precipitated iron oxide and the mixture is heated at 90°C for one hour. During this period, hydrochloric acid is added until the pH of the mixture reaches 7.5. The particles of precipitated iron oxide are washed with deionized water and redispersed in deionized water containing -0.5 g of a potassium salt of a functionalized oligomer (Polywet^{®} KX-4 sold by Uniroyal Chemical) per gram of precipitated iron oxide, by using an ultrasonic probe. Magnetization of the dispersed iron oxide is measured by a Collpits oscillator circuit technique.

### B. Preparation of magnetic latex (Dielectric/ELM absorber)

To a 3-neck flask equipped with a stirrer, two additional funnels and a condenser is added a mixture of 507 g of the 28.5 percent solids dispersion of Fe₃0₄ (200 gauss and average particle size of less than 0.08 pm) and 203 g of deionized water. The mixture is then heated under nitrogen atmosphere to 90°C while stirring the mixture. At this temperature of 90°C, a monomer stream and an aqueous surfactant stream are separately introduced via the two additional funnels into the flask, each stream being introduced at the rate of -6 ml/min over a period of 65 minutes. The monomer stream consists of 64 g of styrene, 16 g of butyl acrylate and 3 g of t-butyl hydroperoxide. The aqueous stream consists of 110 g of deionized water, 2.9 g of the potassium salt of a functionalized oligomer ("Polywet® KX-4") and 2 g of sodium formaldehyde hydrosulfite. The resulting reaction mixture is stirred and maintained under nitrogen at 90°C for an additional half hour. The resulting 25 percent solids latex is concentrated by distillation under vacuum to a 30.3 percent solids latex (dielectric/ELM absorber) having dispersed particles with a polymeric as well as magnetic characteristic. The particles of this latex have a narrow particle size distribution and an average particle diameter of 0.11 pm as determined by hydrodynamic chromatography. The latex remains stable in an applied magnetic field of 1800 gauss and exhibits properties common to magnetic colloids. For example, such magnetic colloids are magnetizable liquids that are instantly demagnitized upon removal of a magnetic field and levitate an object upon application of a magenetic field. Magnetization of the latex by a Collpits oscillator circuit technique, described by E. A. Paterson et al. in the Journal of Colloidal and Interfacial Science, 70, 3 (1977), is estimated to be 135 gauss.

The particles of the latex are recovered by freeze drying the latex at -80°C under vacuum at 0.5 mm Hg.

### C. Preparation of ELM composition (dielectric/ELM absorber/ELM attenuator)

One ELM composition (Sample No. 1) is prepared by dry blending 50.3 g of a dry powder of the aforementioned latex (55.4 percent dielectric/44.6 percent Fe₃0₄) with 33.5 g of carbonyl iron (ELM attenuator) having an average particle size of 3-4 micrometers and sold by GAF Corporation under the trade name Super Fine Special. The blending is carried out on a Brabender mixing apparatus and the resultang blend is then compression molded into flat plates (0.8 cm thicknessx2.6 cm diameter) at 2000 pounds of positive pressure and 230°C for 2 minutes. The sample is cooled to room temperature and the pressure on the sample is released. The resultant plate of the ELM composition is machined into two flat disks having a diameter of 2.54 cm and a thickness of 0.64 cm and 0.32 cm, respectively.

A second ELM composition (Sample No. 2) is prepared following the foregoing procedure using 56.5 g of the dry powder of the latex and 18.8 g of the carbonyl iron. The sample is similarly blended, molded and fabricated into disks. For purposes of comparison, a third sample (Sample No. C) of dry particles of the latex is molded and fabricated into disks by the foregoing procedure.

All of the foregoing samples are tested for ELM absorption and the results are reported in Table 1.

As evidenced by the data in Table I, the compositions of the present invention (Sample Nos. 1 and 2) exhibit significantly better attenuation at a given frequency than does the composition of Sample No. C.

## Claims

1. An electromagnetic absorption composition having a density less than 6 g/cm³ comprising a dielectric matrix having dispersed therein magnetic additives characterized in that the magnetic additives comprise
(1) colloidal-size polymer encapsulated particles of superparamagnetic material as an absorber for electromagnetic radiation and
(2) magnetic particles having a diameter of greater than 1 pm as an attenuator for electromagnetic radiation.

2. The composition of Claim 1 wherein the composition exhibits a magnetic loss tangent greater than 0.05 and an electromagnetic attenuation of greater than 0.5 decibels per centimeter (dB/cm) when the composition having a thickness of 2 centimeters is exposed to electromagnetic radiation having a frequency of 2 Gigahertz.

3. The composition of Claim 2 which has a density in the range from 1.5 to 3 g/cm³ and exhibits a magnetic loss tangent greater than 0.2 and an attenuation greater than 2 dB/cm.

4. The composition of Claim 2 wherein the superparamagnetic material of the absorber is an oxide of a magnetic metal and the attenuator is a magnetic metal or an alloy containing at least one magnetic metal.

5. The composition of Claim 4 wherein the magnetic metal is iron.

6. The composition of Claim 5 wherein the superparamagnetic material of the absorber is Fe₃0₄ having a maximum particle dimension less than 1 pm and the attenuator is carbonyl iron.

7. The composition of Claim 6 wherein Fe₃0₄ has a maximum particle dimension in the range from 0.01 to 0.7 pm and the carbonyl iron has an average particle size in the range from 2 to 40 pm.

8. The composition of Claim 7 comprising from 90 to 15 weight parts of a dielectric synthetic thermoplastic material and from 10 to 85 weight parts of combined absorber and attenuator wherein the weight ratio of absorber to attenuator is from 90:10 to 60:40.

9. The composition of Claim 8 wherein the synthetic thermoplastic material is a styrene/butyl acrylate copolymer.

10. The composition of Claim 7 wherein substantially all of the particles of the absorber and attenuator are maintained in a discrete spaced apart relationship by the thermoplastic.

11. Use of the composition of Claims 1-10 as base for a liquid coating formulation.

## Patentansprüche

1. Elektromagnetische Strahlung absorbierende Zusammensetzung mit einer Dichte von weniger als 6 g/cm³, enthaltend eine dielektrische Matrix mit darin dispergierten magnetischen Zusätzen, dadurch gekennzeichnet, daß die magnetischen Zusätze enthalten
(1) in Polymer eingekapselte Teilchen superparamagnetischen Materials in kolloidaler Größe als Absorber für elektromagnetische Strahlung und
(2) magnetische Teilchen mit einem Durchmesser größer als 1 pm zum Dämpfen elektromagnetischer Strahlung.

2. Zusammensetzung nach Anspruch 1, dadurch gekennzeichnet, daß die Zusammensetzung einen magnetischen Verlustwinkel (tang) größer als 0,05 und eine elektromagnetische Dämpfung von größer als 0,5 Dezibel pro Centimeter (dB/cm) aufweist, wenn die Zusammensetzung mit einer Dicke von 2 cm elektromagnetischer Strahlung mit einer Frequenz von 2 Gigahertz ausgesetzt wird.

3. Zusammensetzung nach Anspruch 2, dadurch gekennzeichnet, daß sie eine Dichte im Bereich von 1,5 bis 3 g/cm³ hat und einen magnetischen Verlustwinkel (tang) größer als 0,2 und eine Dämpfung größer als 2 dB/cm aufweist.

4. Zusammensetzung nach Anspruch 2, dadurch gekennzeichnet, daß das superparamagnetische Material des Absorbers ein Oxid eines magnetischen Metalls und das dämpfende Material ein magnetisches Metall oder eine Legierung ist, die mindestens ein magnetisches Metall enthält.

5. Zusammensetzung nach Anspruch 4, dadurch gekennzeichnet, daß das magnetische Metall Eisen ist.

6. Zusammensetzung nach Anspruch 5, dadurch gekennzeichnet, daß das superparamagnetische Material des Absorbers Fe₃0₄ ist mit einer maximalen Teilchengröße kleiner als 1 um und das dämpfende Material Eisencarbonyl ist.

7. Zusammensetzung nach Anspruch 6, dadurch gekennzeichnet, daß das Fe₃0₄ eine maximale Teilchengröße im Bereich von 0,01 bis 0,7 um aufweist und das Eisencarbonyl eine mittlere Teilchengröße im Bereich von 2 bis 40 um aufweist.

8 Zusammensetzung nach Anspruch 7, dadurch gekennzeichnet, daß es von 90 bis 15 Gewichtsteile eines dielektrischen synthetischen thermoplastischen Materials und von 10 bis 85 Gewichsteile kombinierten Absorbers und dämpfenden Materials enthält, wobei das Gewichtsverhältnis von Absorber:dämpfendem Material von 90:10 bis 60:40 beträgt.

9. Zusammensetzung nach Anspruch 8, dadurch gekennzeichnet, daß das synthetische thermoplastische Material in Styrol/Butylacrylatcopolymer ist.

10. Zusammensetzung nach Anspruch 7, dadurch gekennzeichnet, daß im wesentlichen alle Teilchen des Absorbers und des dämpfenden Materials durch das Thermoplast in diskretem Abstand voneinander gehalten werden.

11. Verwendung der Zusammensetzung nach Ansprüche 1-10 als Basis für eine flüssige Beschichtungszusammensetzung.

## Revendications

1. Composition d'absorption électromagnétique possédant une densité inférieure à 6 g/cm³ et comprenant une matrice diélectrique dans laquelle sont dispersés des additifs magnétiques, caractérisée en ce que les additifs magnétiques, comprenant:
(1) des particules de taille colloïdale, d'une matière superparamagnétique enrobées dans un polymère, servant d'absorbant vis-à-vis des rayonnements électromagnétiques, et
(2) des particules magnétiques d'un diamètre supérieur à 1 µm, servant d'atténuator vis-à-vis des rayonnements électromagnétiques.

2. Composition selon la revendication 1, dans laquelle la composition possède une tangente de l'angle de pertes magnétiques supérieure à 0,05 et une atténuation électromagnétique supérieure à 0,5 décibel par centimère (dB/cm) lorsque la composition, ayant une épaisseur de deux centimètres est soumise à un rayonnement électromagnétique présentant une fréquence de 2 Gigahertz.

3. Composition selon la revendication 2, qui a une densité dans la gamme de 1,5 à 3 g/cm³ et possède une tangente de l'angle de pertes magnétiques supérieure à 0,2 et une atténuation supérieure à 2 dB/cm.

4. Composition selon la revendication 2, dans lequelle la matière superparamagnétique de l'absorbant est un oxyde d'un métal magnétique et l'atténuateur est un métal magnétique ou un alliage contenant au moins un métal magnétique.

5. Composition selon la revendication 4, dans laquelle le métal magnétique est le fer.

6. Composition selon la revendication 5, dans laquelle la matière superparamagnétique de l'absorbant est du Fe₃0₄ possédant une dimension maximale de particules inférieure à 1 um et en ce que l'atténuator est du fer carbonyle.

7. Composition selon la revendication 6, dans laquelle le Fe₃0₄ possède une dimension maximale de particules dans la gamme de 0,01 à 0,7 pm et en ce que le fer carbonyle possède une taille moyenne de particules dans la gamme de 2 à 40 pm.

8. Composition selon la revendication 7, comprenant de 90 à 15 parties en poids d'une matière thermoplastique synthétique diélectrique et de 10 à 85 parties en poids d'absorbent et attènuateur combinés, le rapport en poids de l'absorbant à l'atténuateur étant de 90:10 à 60:40.

9. Composition selon la revendication 8, dans laquelle la matière thermoplastique synthétique est un copolymère styrène/acrylate de butyle.

10. Composition selon la revendication 7, dans laquelle pratiquement toutes les particules de l'absorbant et de l'attènuateur sont maintenues à une distance déterminée les unes des autres par la matière thermoplastique.

11. Utilisation d'une composition selon les revendications 1 à 10 en tant que base pour une formulation de revêtement liquide.
